

## UNITED STATES PATENT OFFICE

2,537,111

TRACING CLOTH AND THE LIKE AND  
METHOD OF PREPARING SAMEHorace Wood, Jr., Wakefield, Mass., assignor to  
Monsanto Chemical Company, St. Louis, Mo., a  
corporation of DelawareNo Drawing. Application July 1, 1948,  
Serial No. 36,443.

14 Claims. (Cl. 117—161)

1

The present invention relates to a method of preparing improved tracing cloth, holland cloth and the like and to the coated articles per se. It more particularly relates to a method of preparing improved tracing cloth and the like which is especially adapted to be sensitized with a photographic emulsion coating.

Tracing cloth has, in general, been manufactured heretofore by first impregnating a woven cotton fabric, fabricated from fine long staple cotton yarns, with a starch-water mixture, after which, the fabric is dried and super-calendered or friction-calendered at a high temperature as, for example, about 410° F. It is not possible to directly coat the starch-impregnated fabric with a photographic gelatin emulsion since the starch is water sensitive and is removed from the fabric to a considerable extent on immersion in water and, therefore, could not suitably withstand the developing and washing processes normally employed in photographic reproduction work. Therefore, in order to employ starch-impregnated fabrics for this use it has been necessary to coat such fabrics with a clear water-resistant film or coating of nitrocellulose, ethyl cellulose or the like antecedent to the application thereto of a photographic emulsion coating.

The foregoing method leaves much to be desired. For example, it is difficult to apply a completely protective nitrocellulose or other water-resistant coating over the starch impregnant. Such a coating is necessary, however, in order to prevent water from swelling the starch and causing image distortion and/or peeling of the protective coating and the like. In practice complete protection of the starch from the water used in the photographic reproduction processes is not always achieved with the result that the photographic reproduction must at times be rejected as not being suitable for its intended use whether it be used as a master print or a copy. The above described method is also relatively inefficient in that extra steps are employed in manufacturing the lacquered tracing cloth, and, therefore, requires the use of considerable extra equipment and labor.

The same difficulties exist in varying degrees in the manufacture of holland cloth, surveying tapes, measuring tapes and the like.

The present invention provides a process for manufacturing tracing cloth, holland cloth and the like, which is not only efficiently and economically carried out, but which also eliminates many of the foregoing and other difficulties and disadvantages in the prior art processes and the products prepared by such processes.

2

It is one object of the present invention to manufacture a tracing cloth, holland cloth and the like for photographic and non-photographic uses by employing a coating impregnant which is not only water-resistant and flexible, but which is also capable of being suitably super-calendered and glazed.

A further object of the invention is to provide a simple and efficient process for manufacturing tracing cloth especially suitable for photographic reproduction uses.

A further object of the invention is to produce by the use of a single impregnant a tracing cloth which is especially adapted to be sensitized with photographic emulsion coatings and which can be processed in water solutions without the use of an additional water-resistant coating.

Still further objects and advantages of the present invention will appear from the following description and the appended claims.

The invention is practiced, in general, by first impregnating a fabric, which is suitable as a base for tracing cloth, holland cloth, measuring tape or the like, with an organic solvent solution comprising as an essential film-forming material a copolymer of a polymerizable vinyl compound having the structural formula  $R-CH=CH_2$ , where R is a phenyl or substituted phenyl radical, with a secondary alkyl half ester of an ethylene  $\alpha,\beta$ -dicarboxylic acid, in which the alkyl group contains from 4 to 12 carbon atoms. The impregnating solution preferably also contains a minor proportion, based on said copolymer, of polyvinyl butyral. After the fabric is impregnated in the manner indicated, it is heated to evaporate the organic solvent or dried in suitable manner and is then friction-calendered or super-calendered using heat and pressure to glaze the film-forming material or materials.

A clear coating is formed by the above procedure, but such coating may be opacified, if desired, by incorporating a small amount of pigment, flattening agent and the like in the impregnation solution. The super-calendered fabric possesses sufficient water-resistance to be employed as a non-sensitized tracing cloth, as holland cloth and the like. When the super-calendered fabric is to be employed in the manufacture of light sensitive tracing cloth and the like, the resistance of the coating thereon to water and organic solvents is preferably improved, however, by incorporating in the impregnating solution a relatively small proportion, say about 0.5 to 5% by weight, of a compound which is capable of cross-linking the carboxyl groups in the copolymer. As examples of such cross-

linking compounds may be mentioned formaldehyde; amino-aldehyde monomeric or low polymeric resins; phenol-formaldehyde monomeric or low polymeric resins; alkylene polyamines such as ethylene diamine, propylene diamine, butylene diamine and the like; and polyglycols such as triethylene glycol, tetraethylene glycol and the like. When the impregnating solution contains such compounds, the film-forming materials described above are at least partially cross-linked or otherwise inter-reacted to produce a film or coating which is substantially resistant to the organic solvents in which they are originally soluble. The cross-linking or mutual reaction of at least a portion of the film-forming materials in the presence of such a cross-linking compound is accelerated by heat and/or an acid type catalyst. It is preferable when the above compounds are employed to heat the supercalendered fabrics at temperatures between about 225° F. to 330° F. in the presence of an acid catalyst such as tartaric acid, ethyl phosphoric acid, oxalic acid, citric acid or the like as, for example, for a period of from 1 to 15 minutes, depending upon the temperature used, to accelerate the cross-linking or curing of the film-forming materials. Normally, the above copolymers and the polyvinyl butyral resin mutually react or cross-link at least partially merely on aging without the use of such cross-linking compounds, but the cross-linking generally proceeds at a relatively slow rate under such conditions.

Of the above described cross-linking compounds or agents, the amino-aldehyde resins are preferably employed. As examples of such resins may be mentioned urea-formaldehyde resins such as methylol urea and di-methylol urea; alkylated urea-formaldehyde resins or alkoxy alkyl urea resins such as methoxy methyl urea, di-(methoxy methyl) urea, (methoxy methyl) methylol urea and the like; melamine-aldehyde resins such as the methylol melamines and particularly those having from 1 to 4 methylol groups per mol of melamine and the like; and alkylated melamine-aldehyde resins or alkoxy alkyl melamine resins such as (methoxy methyl) mono-methylol melamine, di-(methoxy methyl) mono-methylol melamine, di-(methoxy methyl) di-methylol melamine and the like or mixtures thereof. Of these the methyl ethers of methylol melamines or methylated melamine-formaldehyde resins of the type last described are preferred.

The copolymers employed herein as essential film-forming materials may be prepared in a variety of ways, but are generally prepared by copolymerizing by various well-known methods a polymerizable vinyl compound, having the structural formula  $R-\text{CH}=\text{CH}_2$ , where R is a phenyl radical, a halogen substituted phenyl radical such as chloro phenyl, dichlor phenyl and the like, or a methyl substituted phenyl radical such as methyl phenyl, dimethyl phenyl and the like with a secondary half ester of an ethylene  $\alpha,\beta$ -dicarboxylic acid in which the alkyl group contains from 4 to 12 carbon atoms and preferably 6 to 10 carbon atoms. The vinyl compound and half ester are generally copolymerized in a molal ratio varying between about 2:1 to 1:1 and preferably in a molal ratio of 1.5:1 to 1.1:1. The secondary alkyl ester of an ethylene  $\alpha,\beta$ -dicarboxylic acid may also comprise a small proportion of an ethylene  $\alpha,\beta$ -dicarboxylic acid or anhydride.

As examples of such secondary half esters may

be mentioned sec.-butylacid maleate, butylmethyl carbonyl acid maleate, methyl amyl carbonyl acid maleate, methyl hexyl carbonyl acid maleate, methyl heptyl carbonyl acid maleate, methyl decyl carbonyl acid maleate and the like, the corresponding acid fumarates and the like.

The secondary alkyl half esters are prepared, in general, by reacting a secondary alcohol as, for example, secondary butyl alcohol, methyl isobutyl carbinol and the like with an ethylene  $\alpha,\beta$ -dicarboxylic acid or anhydride such as maleic acid, fumaric acid, maleic anhydride and the like. The alcohol and acid or anhydride are preferably reacted in a molal ratio varying between about 1:1 to 1:1.6. The unreacted alcohol, acid or anhydride can be removed or separated from the secondary alkyl ester so formed, if desired, or the entire mass can be employed in the subsequent polymerization with the above described vinyl compounds.

The above described copolymers may be prepared, if the secondary alkyl half ester and vinyl compound are mutually soluble, by mass polymerization which involves heating the reactants or monomers at temperatures varying between about 100° to 300° C., usually, in the presence of a catalyst as, for example, a peroxide catalyst such as benzoyl peroxide. If the half-ester and vinyl compound are not mutually soluble, the copolymer may be prepared, for example, by emulsion polymerizing the monomers or by copolymerizing the monomers in a solvent for the monomers and copolymer. In the latter case the copolymer may be precipitated after it is formed, for example, by adding an inert diluent to the reaction mixture. The precipitated copolymer can then be separated from the mixture by filtration, centrifuging and the like.

The copolymers employed in the present invention are, in general, soluble in a wide variety of organic solvents and solvent mixtures. As examples of these may be mentioned: alcohols such as methanol, ethanol, isopropanol, n-propanol, butanol and the like; esters of acetic acid such as ethyl acetate, propyl acetate, butyl acetate and the like; ketones such as acetone, diethyl ketone, methyl ethyl ketone, methyl isobutyl ketone and the like; mixtures of alcohols or acetates with aromatic or aliphatic hydrocarbons as, for example, such mixtures as ethanol-toluol, propanol-toluol, ethyl acetate-toluol, ethanol-petroleum naphtha fractions; propanol-petroleum naphtha fractions, ethyl acetate-petroleum naphtha fractions and the like. The foregoing solvents, generally speaking, are also solvents for a mixture of the above copolymers, polyvinyl butyral and the above described cross-linking compounds.

Solutions of the above copolymers in the foregoing solvents or solvent mixtures can be applied to a fabric suitable for tracing cloth, holland cloth and the like in various ways as, for example, by knife coating, roll coating, and the like or by immersing the fabric in the solution and then removing the excess solution. Other methods of application may also be employed. The quantity of polymer present in such solution may be varied considerably depending upon the means used to apply the solution to the fabric, the particular end use of the fabric, the viscosity of the copolymer in the solution, the quantity of other film-forming material or compounds of the type hereinbefore described present in the solution etc. In general, from about 5 to 30% by weight

of the copolymer is used in the impregnating solution when such copolymer is present as the sole film-forming material. When, in addition, polyvinyl butyral and/or the above described cross-linking compounds are also employed in the impregnating solution, the solution generally comprises from about 6 to 32% by weight of solids, including the aforementioned copolymers.

The quantity of solids applied by the various impregnating methods described above may be varied considerably depending upon the end use of the impregnated fabric after super-calendering. When the super-calendered fabric is to be employed in the manufacture of light sensitized tracing cloth, for example, an impregnated and super-calendered fabric containing about 35 to 90% by weight of solids, based on the fabric weight, can be suitably used for this purpose.

In a preferred embodiment of the invention polyvinyl butyral and a cross-linking compound or agent of the type hereinbefore described are employed along with the above described copolymers to give improved flexibility and solvent resistance to the tracing cloth. The quantity of polyvinyl butyral present in the impregnating solution depends to a considerable extent on the degree of flexibility desired in the finished cloth or fabric. In general, from about 1 to 35% by weight of polyvinyl butyral, based on the copolymer, is employed in the impregnating solution, while from about 25 to 30% by weight of polyvinyl butyral, based on the copolymer, is preferably employed.

A further understanding of the present invention will be obtained from the following examples which are intended to be illustrative of the invention, but not limitative of the scope thereof, parts and percentages being by weight.

#### Example I

A copolymer (hereinafter referred to as copolymer A) was prepared by first reacting about 1 molecular proportion of methyl isobutyl carbinol with 1.1 molecular proportions of maleic anhydride at a temperature of about 65° C. until the resulting product had a substantially constant acid value on continued heating. The product thus prepared was copolymerized with about 1.5 molecular proportions of styrene in the presence of about 0.003 molecular proportion of benzoyl peroxide. The reaction was initiated at about 70° C. and this temperature was maintained during the period of rapid heat evolution. The temperature of the mass was then raised to 120° C. for a period of 1½ hours to complete the reaction. On cooling, a hard, glassy resin was obtained which was comminuted to make it more readily soluble.

An impregnating solution was made up containing 20 parts of copolymer A (as prepared above) and 80 parts of special denatured alcohol No. 1 and this solution was knife coated onto a bleached cotton woven fabric weighing 1.9 oz. per square yard and having about 85 warp ends and 87 filling yarns per inch. The impregnated fabric was dried at about 110° F. for approximately 5 minutes in a tunnel drier. The other surface of the fabric was then impregnated and dried in a similar manner and the fabric was then friction-calendered using a three roll friction-calender. The friction roll of the calender was rotated at a peripheral velocity 2 times greater than the peripheral velocity of the fabric rolls. During the friction-calendering operation,

a pressure of 14 tons per linear inch on the fabric was employed and the temperature of the rolls was about 310° F. The impregnated fabric was given 3 passes through the calender and was then ready for coating with a photographic emulsion. The surface of the fabric, which had been exposed to the friction roll, had a smooth, highly glazed, slightly opaque finish which was fairly water-resistant.

#### Example II

An impregnating solution was prepared which contained 14 parts of copolymer A (prepared as described in Example I), 6 parts of polyvinyl butyral and 80 parts of special denatured alcohol No. 1. This solution was roll coated onto a bleached cotton fabric weighing 1.9 oz. per square yard and having 85 warp ends and 87 filling yarns per inch. The impregnated fabric was dried at about 100° F. for 10 minutes. The other surface of the fabric was impregnated and dried by a similar procedure and the fabric was then given two passes through a three roll friction-calender. The friction roll of the calender was driven at 3 times the peripheral velocity of the feed rolls. The temperature of the rolls was about 320° F. and the pressure on the fabric was about 15 tons per linear inch. The surface of the fabric which had been exposed to the friction roll was smooth and highly glazed. The tracing cloth so produced was fairly water-resistant and possessed good flexibility.

#### Example III

An impregnating solution was prepared which contained 17.5 parts of copolymer A (prepared as described in Example I), 7.5 parts of polyvinyl butyral, 2.1 parts of an aqueous solution consisting of 60% by weight of di-(methoxymethyl) dimethylol melamine and 72.9 parts of a solvent mixture consisting of 40% special denatured alcohol No. 1 and 60% toluol. This solution was knife coated onto a woven bleached cotton fabric having substantially the same weight and construction as that described in Example I. The fabric was dried at about 115° F. for 5 minutes and the other surface was then impregnated with the solution and dried using the same procedure. The dry impregnated fabric was given three passes through a three roll friction-calender wherein the friction roll was driven at 3 times the peripheral velocity of the feeding rolls. The temperature of the rolls was maintained at about 315° F. and the pressure on the fabric was approximately 13.5 tons per linear inch. The tracing cloth was then heated to a temperature of 250 to 260° F. for a period of 5 minutes to cure or cross-link the film-forming materials.

The cured tracing cloth is highly flexible and resistant to water, alcohol, and alcohol-hydrocarbon mixtures. It is also resistant to other organic liquids which are normally solvents for the copolymer and polyvinyl butyral.

The polyvinyl butyral employed in the foregoing examples was prepared by condensing butyraldehyde with a partially hydrolyzed polyvinyl acetate and contained on a weight basis 17 to 20% hydroxy groups calculated as polyvinyl alcohol, less than 3% acetate groups calculated as polyvinyl acetate and the remainder substantially butyraldehyde acetal. Instead of this specific polyvinyl butyral other polyvinyl butyrals having lower hydroxy contents, higher acetate contents and/or lower viscosity may be employed. In general, the properties of the film formed from

the foregoing copolymers together with polyvinyl butyral as, for example, extensibility, flexibility and hardness will depend to a certain extent on the particular composition of the polyvinyl butyral and the method employed in preparing it. For these reasons, it will be apparent that the impregnating solutions described herein may be modified to a certain extent depending upon the characteristics of the polyvinyl butyral that is employed.

In the foregoing description and examples other conditions of drying and super-calendering the impregnated fabric may be used. For example, the impregnated cloth may be dried at any temperature which drives off the solvent contained in the impregnating solution, but is preferably dried at temperatures which allow the solvent to be released at such a rate whereby formation of blisters or bubbles on the fabric surface is avoided. If speed of drying is unimportant the impregnated fabric can be dried at normal room temperatures. The fabric can be dried satisfactorily, for example, at temperatures varying between about 90° to 120° F.

Calendering may be carried out by using other means and conditions than those described above. For example, the dried impregnated fabric may be super-calendered by hand ironing using a hot iron to cause thermoplastic flow of the copolymer and polyvinyl butyral, if the latter is also employed. When super-calendering is effected by friction-calendering the various conditions of operating the friction calender may be varied depending upon the type of apparatus employed and the end use of the impregnated and calendered fabric. In general, the impregnated fabric is super-calendered at temperatures and pressures which will cause the copolymer to soften or flow into a substantially continuous film or surface. Suitable temperatures for super-calendering vary between about 275 to 330° F., while temperatures of about 310 to 325° F. are preferably employed. However, other temperatures may be used depending upon the particular copolymer used and the ratio of copolymer to polyvinyl butyral employed in the impregnating solution.

What is claimed is:

1. A method of producing tracing cloth which comprises impregnating a woven cotton fabric which is suitable as a base for tracing cloth with an organic solvent solution comprising (1) from 5 to 30% by weight of a copolymer consisting of a secondary alkyl half ester of an ethylene  $\alpha,\beta$  dicarboxylic acid selected from the group consisting of maleic and fumaric acids, and a polymerizable vinyl compound having the structural formula: R—CH=CH<sub>2</sub>, where R is selected from the group consisting of a phenyl, halogen substituted phenyl and methyl substituted phenyl radical, said half ester and said vinyl compound being copolymerized in a molal ratio between 1:1 and 1:2, (2) a minor proportion, based on said copolymer, of polyvinyl butyral, (3) from 0.5 to 5% by weight of a compound selected from the group consisting of formaldehyde, phenol-formaldehyde resins, urea-aldehyde resins, alkoxy alkyl urea resins, melamine-aldehyde resins, alkoxy alkyl melamine resins, alkylene polyamines and polyglycols and (4) an organic solvent for the foregoing ingredients, said solution comprising from 6 to 32% by weight of solids; drying said fabric and then friction-calendering said fabric.

2. A method of producing tracing cloth which comprises impregnating a woven cotton fabric which is suitable as a base for tracing cloth with

an organic solvent solution comprising (1) from 5 to 30% by weight of a copolymer consisting of a secondary alkyl half ester of an ethylene  $\alpha,\beta$  dicarboxylic acid selected from the group consisting of maleic and fumaric acids, in which the alkyl group contains from 4 to 12 carbon atoms, and styrene, said half ester and styrene being copolymerized in a molal ratio between 1:1 and 1:2, (2) a minor proportion, based on said copolymer, of polyvinyl butyral, (3) from 0.5 to 5% by weight of a compound selected from the group consisting of formaldehyde, phenol-formaldehyde resins, urea-aldehyde resins, alkoxy alkyl urea resins, melamine-aldehyde resins, alkoxy alkyl melamine resins, alkylene polyamines and polyglycols and (4) an organic solvent for the foregoing ingredients, said solution comprising from 6 to 32% by weight of solids; drying said fabric and then friction-calendering said fabric.

20 3. A method of producing tracing cloth which comprises impregnating a woven cotton fabric which is suitable as a base for tracing cloth with an organic solvent solution comprising (1) from 5 to 30% by weight of a copolymer consisting of a secondary alkyl half ester of an ethylene  $\alpha,\beta$  dicarboxylic acid selected from the group consisting of maleic and fumaric acids, in which the alkyl group contains from 6 to 10 carbon atoms, and styrene, said half ester and styrene being copolymerized in a molal ratio between 1:1 and 1:2, (2) a minor proportion, based on said copolymer, of polyvinyl butyral, (3) from 0.5 to 5% by weight of a methyl ether of methylol melamine and (4) an organic solvent for the foregoing ingredients, said solution comprising from 6 to 32% by weight of solids; drying said fabric and then friction-calendering said fabric.

25 4. A method according to claim 3, but further characterized in that the secondary alkyl half ester is methyl isobutyl carbonyl acid maleate.

40 5. A method according to claim 3, but further characterized in that the secondary alkyl half ester is methyl amyl carbonyl acid maleate.

45 6. A method according to claim 3, but further characterized in that the secondary alkyl half ester is methyl hexyl carbonyl acid maleate.

50 7. A friction-calendered tracing cloth which consists essentially of a woven cotton fabric suitable as a base for tracing cloth impregnated with a copolymer consisting of a secondary alkyl half ester of an ethylene  $\alpha,\beta$  dicarboxylic acid selected from the group consisting of maleic and fumaric acids, and a polymerizable vinyl compound having the structural formula: R—CH=CH<sub>2</sub>, where R is a member of the class consisting of a phenyl, halogen substituted phenyl and methyl substituted phenyl radical, said half ester and said vinyl compound being copolymerized in a molal ratio between 1:1 and 1:2.

55 8. A friction-calendered tracing cloth which consists essentially of a woven cotton fabric suitable as a base for tracing cloth impregnated with (1) a copolymer consisting of a secondary alkyl half ester of an ethylene  $\alpha,\beta$  dicarboxylic acid selected from the group consisting of maleic and fumaric acids, and a polymerizable vinyl compound having the structural formula: R—CH=CH<sub>2</sub>, where R is selected from the group consisting of a phenyl, halogen substituted phenyl and methyl substituted phenyl radical, said half ester and said vinyl compound being copolymerized in a molal ratio between 1:1 and 1:2, and (2) a minor proportion, based on said copolymer, of polyvinyl butyral.

9. A friction-calendered tracing cloth which consists essentially of a woven cotton fabric suitable as a base for tracing cloth impregnated with (1) a copolymer consisting of a secondary alkyl half ester of an ethylene  $\alpha,\beta$  dicarboxylic acid selected from the group consisting of maleic and fumaric acids, and a polymerizable vinyl compound having the structural formula:



where R is selected from the group consisting of a phenyl, halogen substituted phenyl and methyl substituted phenyl radical, said half ester and said vinyl compound being copolymerized in a molal ratio between 1:1 and 1:2, (2) a minor proportion, based on said copolymer, of polyvinyl butyral and (3) a small proportion of a compound selected from the group consisting of formaldehyde, phenol-formaldehyde resins, urea-aldehyde resins, alkoxy alkyl urea resins, melamine-aldehyde resins, alkoxy alkyl melamine resins, alkylene polyamines and polyglycols, said copolymer, butyral and last named compound being at least partly inter-reacted.

10. A friction-calendered tracing cloth which consists essentially of a woven cotton fabric suitable as a base for tracing cloth impregnated with (1) a copolymer consisting of a secondary alkyl half ester of an ethylene  $\alpha,\beta$  dicarboxylic acid selected from the group consisting of maleic and fumaric acids, in which the alkyl group contains from 4 to 12 carbon atoms, and styrene, said half ester and styrene being copolymerized in a molal ratio between 1:1 and 1:2, (2) a minor proportion, based on said copolymer, of polyvinyl butyral and (3) a small proportion of a compound selected from the group consisting of formaldehyde, phenol-formaldehyde resins, urea-aldehyde resins, alkoxy alkyl urea resins, melamine-aldehyde resins, alkoxy alkyl melamine resins, alkylene polyamines and polyglycols, said copolymer, butyral and last named compound being at least partly inter-reacted.

11. A friction-calendered tracing cloth which consists essentially of a woven cotton fabric suitable as a base for tracing cloth impregnated with (1) a copolymer consisting of a secondary alkyl half ester of an ethylene  $\alpha,\beta$  dicarboxylic acid selected from the group consisting of maleic and fumaric acids, in which the alkyl group contains from 6 to 10 carbon atoms, and styrene, said half ester and styrene being copolymerized in a molal ratio between 1:1 and 1:2, (2) a minor proportion, based on said copolymer, of polyvinyl butyral and (3) a small proportion of a methyl ether of methylol melamine, said copolymer,

10  
15

butyral and methyl ether being at least partly inter-reacted.

12. A friction-calendered tracing cloth which consists essentially of a woven cotton fabric suitable as a base for tracing cloth impregnated with (1) a copolymer consisting of methyl isobutyl carbonyl acid maleate and styrene, said maleate and styrene being copolymerized in a molal ratio between 1:1 and 1:2, (2) a minor proportion, based on said copolymer, of polyvinyl butyral and (3) a small proportion of a methyl ether of methylol melamine, said copolymer, butyral and methyl ether being at least partly inter-reacted.

13. A friction-calendered tracing cloth which consists essentially of a woven cotton fabric suitable as a base for tracing cloth impregnated with (1) a copolymer consisting of methyl amyl carbonyl acid maleate and styrene, said maleate and styrene being copolymerized in a molal ratio between 1:1 and 1:2, (2) a minor proportion, based on said copolymer, of polyvinyl butyral and (3) a small proportion of a methyl ether of methylol melamine, said copolymer, butyral and methyl ether being at least partly inter-reacted.

14. A friction-calendered tracing cloth which consists essentially of a woven cotton fabric suitable as a base for tracing cloth impregnated with (1) a copolymer consisting of methyl hexyl carbonyl acid maleate and styrene, said maleate and styrene being copolymerized in a molal ratio between 1:1 and 1:2, (2) a minor proportion, based on said copolymer, of polyvinyl butyral and (3) a small proportion of a methyl ether of methylol melamine, said copolymer, butyral and methyl ether being at least partly inter-reacted.

HORACE WOOD, JR.

#### REFERENCES CITED

40 The following references are of record in the file of this patent:

#### UNITED STATES PATENTS

| Number.   | Name        | Date          |
|-----------|-------------|---------------|
| 2,047,398 | Voss et al. | July 14, 1936 |
| 2,279,881 | D'Alelio    | Apr. 14, 1942 |
| 2,312,623 | Brooks      | Mar. 2, 1943  |
| 2,377,231 | Hayes       | May 29, 1945  |
| 2,416,232 | Soday       | Feb. 18, 1947 |
| 2,432,232 | Leekley     | Dec. 9, 1947  |
| 2,453,308 | Dunlop      | Nov. 9, 1948  |

#### FOREIGN PATENTS

| Number  | Country       | Date         |
|---------|---------------|--------------|
| 466,898 | Great Britain | June 8, 1937 |